

(No Model.)

C. J. EAMES.

REDUCTION OF IRON ORE.

No. 404,181.

Patented May 28, 1889.



Witnesses:

Fred D. Cornwally  
E. Walker

Inventor:

Charles J. Eames

# UNITED STATES PATENT OFFICE.

CHARLES J. EAMES, OF NEW YORK, N. Y.

## REDUCTION OF IRON ORE.

SPECIFICATION forming part of Letters Patent No. 404,181, dated May 28, 1889.

Application filed January 19, 1889. Serial No. 296,836. (No model.)

*To all whom it may concern:*

Be it known that I, CHARLES J. EAMES, a citizen of the United States, residing at New York city, in the State of New York, have invented certain new and useful Improvements 5 in the Reduction of Iron Ore for the Manufacture of Iron and Steel Direct from the Ore; and I hereby declare the following to be a full, clear, and exact description of the same, 10 such as will enable others skilled in the art of metallurgy to apply the invention.

Heretofore in the reduction of iron ores, especially by such processes as the blast-furnace or stack process and allied processes, 15 where the flame or heated gases came in direct contact with or permeated the mass under treatment, or where the heated gases, flame, &c., swept over and reverberated on the mass to be treated, as in the hearth- 20 reverberatory or roasting processes, it has been the practice to mingle with the carbon or reducing agent and the ore a flux of some character, or to employ a coating or protective covering to prevent too rapid combustion of 25 the carbon; and this has heretofore been deemed essential to a successful working wherever coke, soft or hard coal, or any equivalent reducing agent which combined with oxygen readily and at a low temperature has 30 been employed.

The object I have in view is to dispense with any flux—such as lime or its equivalent—or any protecting coating or other medium for the protection of the carbon or retardation of its combustion, and employ only coke, soft or hard coal, and similar soft carbons intermingled with the ore to be reduced in all such processes as apply the heat by gases which pass over and through the mass 40 to be treated, whereby the reduction process is simplified, impurities prevented from entering the metal, and shortness or brittleness of the iron avoided.

To this end the invention, generally stated, 45 may be said to consist in subjecting layers composed of a mixture of coke, hard coal, or their equivalents—carbons which oxidize at a low temperature—(arranged alternately with layers of carbon alone,) to heated carbonic 50 oxide or equivalent neutral gases which per-

meate the mass, all as will hereinafter more fully appear.

I will now proceed to describe more specifically the preferred manner of applying my invention, and for facility in doing the same 55 I have illustrated apparatus suitable therefor, in which—

Figure 1 is a vertical section of a reducing-stack. Fig. 2 is an elevation of said reducing-stack; and Fig. 3 is a sectional plan view on 60 the line *x x*, Fig. 1, showing the drop-grate.

Like letters refer to like parts wherever they occur.

Any suitable apparatus may be employed. That shown answers the purpose as well as 65 any I know of. It consists of an outer shell, 1, of boiler-plate, of, say, five (5) feet diameter at the base and three (3) feet diameter at the top, or any other desired taper which will permit the charge to drop out freely when the 70 grate of the stack is let down. This shell 1 is supported on a square arched base, 2, is lined with fire-brick, as at 3, and provided with a drop-grate, 4, which may be of two sections hinged at the side, so as to fall away 75 from the center, and a chamber, 5, is formed below the grate by means of a slide, 6, which can be drawn out to obtain a natural draft for the stack.

7 indicates a blast-pipe communicating with 80 chamber 5, and said pipe should have a suitable valve.

8 8 indicate a series of small openings or ports at the base of the stack, which may be closed by doors or by plugs of fire-brick, as 85 preferred.

9 indicates a damper controlled by a chain, 10, and which may be used to close the top of the stack when drawing the charge, so as to avoid drafts over the heated reduced ore after 90 it has been discharged.

The blast 7 is only provided to meet emergencies and prevent scaffolding of the charge in case the stack works irregularly from any cause.

The direct or natural draft obtained by means of the slide 6 is only used in starting the fire or inducing primary incandescence in the lowest strata or base-strata of carbon, the ports 8 8 being used to maintain the slow 100

combustion upon which the process itself depends.

In carrying out my process of reduction I first form a base or bed stratum, A, of lump carbon, which may be of coke—such as Connellsville coke—or graphitic carbon—such as is found at Cranston, Rhode Island, and in other localities—the lumps to be of such size as to give an open or reticulated character to the stratum—say from three to five inches in diameter—and the stratum to be about six (6) or eight (8) inches thick. This stratum A is then ignited, and by means of the natural draft produced by withdrawing slide 6 or by the use of blast 7 is brought to a highly-incandescent condition, more carbon being added from time to time, if desired or required, to preserve the desired depth of said stratum A. For purposes of starting ignition in stratum A wood or other kindling may be used below the stratum, as in building an ordinary fire.

When the stack is thoroughly heated and stratum A thoroughly ignited, the draft or blast is cut off, and the ore to be reduced, in a granulated condition, admixed with carbon in a like condition, is to be charged into the stack as follows: Upon the bed stratum A, I place a stratum, a, of the material to be treated, said stratum composed of an admixture of from twenty (20) to forty (40) per cent. of granulated carbon—such as coke, hard coal, graphitic carbon, (hereinbefore referred to,) or their equivalents—and the iron ore in a like granulated condition—about the size of a grain of wheat—said stratum a to be from two (2) to four (4) inches in thickness. Above the stratum a, I place a stratum, b, composed of carbon only, of any of the forms above mentioned, in lump form, so as to preserve an open or reticulated structure readily permeable by the gases, said stratum b to correspond in thickness to the stratum a—that is to say, from two (2) to four (4) inches thick. I then add alternate layers of the admixed carbon iron ore in granular form (a' a<sup>2</sup> a<sup>3</sup>, &c.) and lump carbon alone (b' b<sup>2</sup> b<sup>3</sup>, &c.) until the stack is filled to within six or eight inches of the top. When the stack is thus charged, I open a sufficient number of the ports 8 8 opposite the bed-stratum A to admit sufficient air to induce low combustion in the bed-stratum A, and the highly-heated neutral

carbonic oxide thus formed will permeate the layers a b a' b', &c., producing a steady and uniform reduction of the iron ore without unduly consuming or exhausting the carbon contained in the strata.

By examining the top layer or stratum of iron ore, &c., it can readily be determined when the reduction of the iron ore is complete by the agglutination of the particles and other characteristics well known to the skilled operator. The damper 9 and the ports 8 8 are then closed, the slide 6 withdrawn, and the grate 4 lowered to dump the charge of reduced ore into the pit or space below the arches. The atmosphere of carbonic oxide which surrounds it will prevent oxidation of the sponge while cooling, and the unconsumed carbon from strata b b' b<sup>2</sup>, &c., can be separated from the mass and used to form the bed-stratum A of the next charge.

Having thus described my invention, what I claim, and desire to secure by Letters Patent, is—

1. The process herein described for reducing iron ores, which consists in subjecting alternately-arranged strata or layers of carbon and granulated iron ore and carbon in admixture to currents of heated carbonic oxide, which are caused to permeate said strata, substantially as and for the purposes specified.

2. The process herein described for reducing iron ore, which consists in subjecting alternately-arranged strata or layers of carbon and granulated iron ore admixed with carbon to currents of heated carbonic oxide, which are formed in a base-strata of carbon and which permeate the superimposed strata of iron ore, &c., substantially as and for the purposes specified.

3. As a step in the herein-described process of reducing iron ore, the arrangement of a bed-strata of graphitic carbon as a means of generating carbonic oxide, and a series of superimposed alternate layers of carbon alone and an admixture of carbon and iron ore, substantially as and for the purposes specified.

In testimony whereof I affix my signature, in presence of two witnesses, this 19th day of January, 1889.

CHARLES J. EAMES.

Witnesses:

E. T. WALKER,  
F. R. CORNWALL.